

# UNITED STATES PATENT OFFICE.

WILLEM VAN DER HEYDEN, OF NANTERRE, FRANCE.

## EMULSIONING AND SOLIDIFICATION OF HYDROCARBONS.

No. 857,425.

Specification of Letters Patent.

Patented June 18, 1907.

Application filed June 23, 1906. Serial No. 323,458.

*To all whom it may concern:*

Be it known that I, WILLEM VAN DER HEYDEN, physician, and a citizen of France, residing at 21 Boulevard du Midi, in the city of

Nanterre, Seine, near Paris, in the Republic of France, have invented a new and useful Improvement in the Emulsioning and Solidification of Hydrocarbons, such as Petroleum, Benzin, Mineral Oils, &c., of which the following is a specification.

It is known by the applicant's German patent No. 176,366 that, fluid hydrocarbons such as kerosene, crude oil, residual oil or benzin, can be emulsionized by means of a solution of glue (colla, glutin, gelatin), and this emulsion can then be solidified by completely drying or hardening the solid blocks with formaldehyde, tannic or chromic acid and such like. I have now found that into this emulsion dustlike fuels can be included, provided, that the quantity of same does not exceed the limits beyond which it is possible to obtain a true emulsion; 30—40% of coal dust or powder can always be bound. The blocks, thus obtained by means of a solution of glue only, show the deficiency that especially the lighter hydrocarbons are not secured from gradually volatilizing when the blocks are stored for some time, a fact, which is, of course detrimental. On the other hand the solidified heavier products of the distillation from the crude oil, such as mineral oil, residual oil and also the crude oil itself, show the disadvantageous property, that for a long time the solid blocks exude resin-like substances. Moreover the blocks manufactured only with glue burn with considerable of smoke if the access of air is not sufficient. These deficiencies can be removed by the addition of further different substances to the emulsion, that is the addition of glycerin in order to prevent the loss of weight of which product 3—4% are sufficient. An addition of salts of organic acids, e. g. of tartaric, oxalic and citric acid effects a smokeless burning of the solidified blocks. The whole process is performed as follows: About 1000 g. of benzin or kerosene or crude oil are emulsioned with 50—60 g. of glue soaked in water and then dissolved by heating on a warm waterbath and with 300—400 g. of dustlike fuels such as coal dust or powder, the hydrocarbon being added to it in

small portions and shaken or querled, until all has become a perfect emulsion and no constituent separates from it after the shaking ceases.

If it is desired to prevent a volatilization of the hydrocarbon 30—40 g. of glycerin are added before emulsioning the mixture. Also 40—50 g. of tartrate or oxalate of potassium are equally added if it is desired to make products burning without smoke. During the emulsioning it is advisable to keep the fluid warm, so that the mixture remains liquid. After all hydrocarbons are well emulsioned the emulsion is poured out into molds of any description and allowed to cool down, if necessary by artificial cooling. The emulsion then very easily becomes hard and can be taken out of the molds. The further hardening process can be effected by drying at the open air, it is, however, more advantageous to harden the glue by means of formaldehyde or tannic or chromic acid, or by alcohol or such like means. The hardening with formaldehyde is performed either by putting the blocks into a watery solution of formaldehyde or by the action of gaseous formaldehyde in an air-tight box. Thus manufactured solidified hydrocarbons with the addition of dustlike fuels represent solid blocks. If they are manufactured with glycerin also, they are considerably elastic and remain absolutely unvariable; even, when stored for many months no loss of weight can be found. Heavy oils such as crude oil, residual oil this solidified are obtained so fast, that the blocks can be stored about 5 meter high without a changing of form or loss of oil. The blocks thus obtained can be lighted only by a flame, not by heat or glowing materials and the flame can easily be extinguished by application of water e. g. by a vaporizer. They can also be kindled again immediately after extinguishing, the water not wetting them. Likewise they are neither affected by moisture nor by heat or cold, even boiling water has no influence at all upon this product. It is very easily handled, does not break or crumble and will burn away almost without any ash.

What I claim and desire to secure by Letters Patent of the United States is:—

1. Improvement in the solidification of hydrocarbons such as naphtha, petroleum,

benzin, benzol and such like, which consists in adding dust-like fuels, such as coal dust and such like, to an emulsion of hydrocarbons and a solution of glue and then submitting the mass to a hardening process.

2. Improvement in the solidification of hydrocarbons such as naphtha, petroleum, benzin, benzol and such like, which consists in adding glycerin and dust-like fuels to an emulsion of hydrocarbons and a solution of glue and then submitting the mass to a hardening process.

3. Improvement in the solidification of hydrocarbons such as naphtha, petroleum, benzin, benzol and such like, which consists in adding salts of organic acids, such as tartrate, oxalate, citrate and dust-like fuels to an emulsion of hydrocarbons and a solution

of glue and then submitting the mass to a hardening process.

4. Improvement in the solidification of hydrocarbons such as naphtha, petroleum, benzin, benzol and such like, which consists in adding glycerin, salts of organic acids, such as tartrate, oxalate, citrate and dust-like fuels to an emulsion of hydrocarbons and a solution of glue and then submitting the mass to a hardening process.

In witness whereof, I have hereunto signed my name in the presence of two subscribing witnesses.

WILLEM VAN DER HEYDEN.

Witnesses:

HERNANDO DE SOTO,  
AUGUSTUS E. INGRAM.